

April 18, 1933.

R. S. DEAN

1,904,859

FERROUS ALLOY

Filed March 24, 1930

3 Sheets-Sheet 1



Inventor  
R. S. Dean

By J. G. Roberts Atty.

April 18, 1933.

R. S. DEAN

1,904,859

FERROUS ALLOY

Filed March 24, 1930

3 Sheets-Sheet 2



Inventor  
R. S. Dean

By J. G. Roberts Atty.

April 18, 1933.

R. S. DEAN

1,904,859

FERROUS ALLOY

Filed March 24, 1930

3 Sheets-Sheet 3



Inventor  
R. S. Dean

By J. G. Roberts Atty.

## UNITED STATES PATENT OFFICE

REGINALD S. DEAN, OF WASHINGTON, DISTRICT OF COLUMBIA, ASSIGNOR TO WESTERN ELECTRIC COMPANY, INCORPORATED, OF NEW YORK, N. Y., A CORPORATION OF NEW YORK

## FERROUS ALLOY

Application filed March 24, 1930. Serial No. 438,263.

REISSUED

This invention relates to ferrous alloys and methods of producing the same, and more particularly to alloys of iron with tungsten, molybdenum, beryllium, and tantalum, and to methods of treating such alloys so as to produce certain desirable mechanical and magnetic characteristics.

An object of the invention is to provide an alloy in which certain desirable physical and magnetic properties are produced by special treatment.

In accordance with the general features of the invention as embodied in one specific form thereof, a quantity of iron, preferably substantially free of carbon, is alloyed with one or more of the above named alloy ingredients, and the mass is then cast in the form of ingots, which are then formed by forging or other means into any desired shape, or such shapes may if desired be formed directly from the molten metal. The forgings are then heated to a temperature just below the eutectic point of the alloy, and this temperature is maintained for a sufficiently long period of time to cause substantially all of the resulting solute constituent to enter solution in the iron, and the alloy is then quenched at a sufficiently rapid rate to cause the solute constituent to remain in the iron in the form of a supersaturated solid solution, after which the alloy is caused to assume a more stable state by aging. The hardness of the alloy as quenched may be increased considerably by such aging, and the secondary hardness is retained even at elevated temperatures. In the manufacture of articles such as dies or permanent magnets from alloys of the type just described, an article may be forged or otherwise formed from the alloy and the formed article then subjected to the above outlined heating, cooling, and aging operations.

The above described and other objects and features of the invention will be apparent from the following detailed description, taken in connection with the accompanying drawings, in which

Fig. 1 is a graphic representation of certain phenomena encountered in the aging of an

iron-tungsten alloy containing 21.1% of tungsten;

Fig. 2 is a similar representation of the properties of an iron-molybdenum alloy containing 23.4% of molybdenum; 55

Fig. 3 is a similar representation of the properties of an iron-beryllium alloy containing 2.8% of beryllium;

Fig. 4 is a similar representation of the properties of an iron-tantalum alloy containing 24% of tantalum; 60

Fig. 5 is a similar representation of the properties of a quaternary alloy containing approximately 25.7% cobalt, 20.1% tungsten, 6.4% manganese, and the remainder iron. 65

This invention is based on the discovery that the mechanical properties of the above named alloys, as well as the magnetic remanence and coercive force, may be greatly increased by a proper heat treating process, 70 and the magnetic characteristics of the alloy will not necessarily vary with its physical hardness.

Although it is not known with certainty what the solute constituents of these alloys are, it is believed that the alloy ingredient combines chemically with a part of the iron to form a compound which remains in a dispersed phase throughout the iron and may under certain conditions be precipitated in 80 the form of microscopic or submicroscopic particles dispersed throughout the alloy. The various steps constituting the processes described below are the same regardless of whether the alloy ingredient is dissolved in 85 the iron as an element or as a compound, and it is to be understood, therefore, that in the following description and appended claims the term "solute constituent" may include the alloy ingredient either combined or uncombined as the case may actually be. 90

In practicing one method of producing alloys in accordance with the invention, a quantity of tungsten, molybdenum, beryllium or tantalum greater than that which 95 will enter solution in iron at room temperature, but not substantially more than is soluble at the eutectic temperature, is alloyed with iron and the resulting alloy is caused to solidify. The alloy is then heated at a 100

temperature dependent upon which alloy ingredient is used until a substantially homogeneous solid solution is formed, and is then quenched at a rate sufficiently rapid to cause 5 most or all of the alloy ingredient to be retained in the iron in the form of a supersaturated solid solution, and the alloy is subsequently aged at a temperature considerably below the eutectic temperature. The 10 proper length of time and temperature of the solution forming step, quenching or supersaturating step, and the aging step, wherein the alloy is allowed to assume a more stable state, together with the proper proportions of iron and alloy ingredient, will 15 vary with the properties desired in the alloy and the uses to which the alloy is to be put as well as with the particular alloy ingredient employed. However, the following example 20 has been found to produce a satisfactory alloy for permanent magnets. To a substantially carbon-free iron is added 21.1 parts of tungsten, and the two ingredients are agitated in any known manner while in 25 the molten state to produce a homogeneous alloy. The alloy is then cast into ingots and fabricated into desired shapes, which are then brought to a temperature (about 2600° F. in the case of tungsten) slightly below the 30 eutectic temperature, and maintained at such temperature for a sufficient time to produce a solid solution of the tungsten in the iron. The parts are then quickly cooled by quenching, thus producing a solid solution of the 35 solute constituent in the iron. The parts are then heated to about 1400° F., and maintained at such temperature for a time varying from fifteen minutes to an hour, after which they are quenched either rapidly or slowly, the 40 rate of cooling being immaterial. The alloy, after this treatment, will be found to have a magnetic remanence or coercive force higher than that of iron-tungsten alloys heretofore produced, and is suitable for use 45 in permanent magnets. Referring to the drawings, curve B of Fig. 1 indicates the magnetic remanence obtained by treating the alloy at various temperatures for one hour, cooling, and then subjecting the parts 50 to a magnetizing force of 1000 giberts per centimeter. The coercive force is indicated in curve C, and mechanical hardness in curve A. All these characteristics are at 55 or near a maximum when the alloy is aged at about 1400° F. An alloy aged at that temperature, in addition to having desirable magnetic characteristics, is suitable for use 60 in dies for die casting machines and for analogous uses since it is capable of withstanding high temperatures without losing its hardness.

Fig. 2 illustrates the behavior of an iron-molybdenum alloy containing 23.4% of molybdenum, curve D representing the variation in hardness while curves E and F repre-

sent remanence and coercive force respectively. This alloy behaves similarly in most respects to the iron-tungsten alloy above discussed.

Fig. 3 illustrates the behavior of an iron-beryllium alloy containing 2.8% of beryllium, curve G representing the variation in hardness while curves H and I represent remanence and coercive force respectively. It will be noted that in the case of this alloy 70 the remanence reaches its maximum value at a considerably higher aging temperature than the coercive force and hardness.

Fig. 4 illustrates the behavior of an iron-tantalum alloy containing 21.9% of tantalum, 75 curve J representing the variation in hardness while curves K and L represent remanence and coercive force respectively, all of which characteristics reach their maxima at or near 1300° F.

Fig. 5 illustrates the behavior of a quaternary alloy containing approximately 25.7% cobalt, 20.1% tungsten, 6.4% manganese, and the remainder substantially carbon-free iron. The figure shows that the mechanical hardness, represented by curve M, reaches a maximum when the alloy is aged at a temperature of about 1100° F., whereas the remanence, represented by curve N, and the coercive force, represented by curve O, reach 90 their maximum values at considerably higher aging temperatures. The figure also illustrates the possibility of adding alloy ingredients in addition to tungsten, molybdenum, beryllium, and/or tantalum to improve 95 the mechanical characteristics of the alloy, even though the additional alloy ingredients do not themselves form age-hardenable alloys with iron.

Alloys produced in accordance with the 105 process herein disclosed may be used for a variety of other purposes, and it is within the scope of this invention to add to the alloy more than one of the above named metals, as well as such other ingredients as may be 110 found desirable to adapt the alloy to the special purposes to which it is to be put, thus producing ternary and quaternary alloys having such special properties as are necessary to meet special requirements.

It is to be understood that the invention is not limited to the precise temperatures and proportions mentioned herein, which may be varied considerably without departing from the spirit of the invention as defined in the 115 appended claims.

What is claimed is:

1. The method of producing a permanent magnet which comprises alloying a metal of the group including tungsten, molybdenum, beryllium, and tantalum with substantially carbon-free iron, forming a magnet of the 125 alloy, heating the alloy to form a substantially homogeneous solid solution, cooling the solution at a rate to form a supersaturated 130 solution.

solution, heat treating the magnet to develop its magnetic properties, and subjecting the magnet to a magnetizing force to magnetize the magnet.

5 2. A magnetic alloy of a substantially carbon-free iron with substantially 21.1% tungsten in which the tungsten is present in supersaturated solution and heat treated at a temperature of substantially 1400° F. to develop 10 its optimum magnetic properties.

3. A magnetic alloy of a substantially carbon-free iron with substantially 23.4% molybdenum in which the molybdenum is present in supersaturated solution and heat treated at a temperature of substantially 1200° F. to develop its optimum magnetic properties.

4. A magnetic alloy of substantially carbon-free iron with substantially 2.8% beryllium, in which the beryllium is present in supersaturated solution and heat treated at a temperature between 1000° and 1200° F. to develop its optimum magnetic properties.

5. A magnetic alloy of substantially carbon-free iron with substantially 21.9% of tantalum in which the tantalum is present in supersaturated solution and heat treated at a temperature between 1200° and 1400° F. to develop its optimum magnetic properties.

30 6. An alloy of substantially carbon-free iron with approximately 25% cobalt, 20% tungsten, in which the tungsten is present in supersaturated solution, heat-treated at a temperature of substantially 1400° F. to age-harden the alloy.

7. An alloy of substantially carbon-free iron with approximately 25% cobalt, 23% molybdenum, in which the molybdenum is present in supersaturated solution, heat-treated at a temperature of substantially 1300° F. to age-harden the alloy.

8. An alloy of substantially carbon-free iron with approximately 25% cobalt, and a metal of the group of tungsten, molybdenum, beryllium and tantalum, having the metal of the group present in supersaturated solution and heat-treated to age-harden the alloy.

9. A method of making an alloy which comprises alloying iron with cobalt and a metal of the group of tungsten, molybdenum, beryllium, and tantalum, heating the alloy to substantially the eutectic temperature of the metal of the group, quenching the alloy to produce a supersaturated solution of the metal of the group in the alloy, and age-hardening the alloy at a temperature to disperse the metal of the group in the alloy.

10. A method of making an alloy which comprises alloying iron with cobalt and tungsten in which the cobalt is present in the order of 25% and tungsten in the order of 20%, heating the alloy to a temperature of approximately 2600° F. to form a solid solution of the tungsten in the alloy, quenching the alloy to form a supersaturated so-

lution of the tungsten in the alloy, and age-hardening the alloy at a temperature of approximately 1400° F.

11. A method of making an alloy which comprises alloying iron with cobalt and molybdenum in which the cobalt is present in the order of 25% and molybdenum in the order of 23%, heating the alloy to a temperature of approximately the eutectic temperature of molybdenum to form a solid solution of the molybdenum in the alloy, quenching the alloy to form a supersaturated solution of the molybdenum in the alloy, and age-hardening the alloy at a temperature of approximately 1300° F.

12. A method of making an alloy which comprises alloying iron with cobalt, magnesium, and a metal of the group of tungsten, molybdenum, beryllium, and tantalum, heating the alloy to substantially the eutectic temperature of the metal of the group to form a solid solution of the metal of the group in the alloy, quenching the alloy to form a supersaturated solution, and age-hardening the alloy to disperse the metal of the group in the alloy.

In witness whereof, I hereunto subscribe my name this 3rd day of March A. D., 1930.

REGINALD S. DEAN.

70

80

85

90

95

100

105

110

115

120

125

130